# EUROPEAN PATENT SPECIFICATION

(11) **EP 0 021 850 B1**
(45) Date of publication and mention of the grant of the patent: **27.07.1983**
(21) Application number: 80302219.3
(22) Date of filing: 01.07.1980
(51) Int. Cl.: C25C 3/08, C25D 3/66

(54) **Alumina reduction cell, methods of producing such a cell, and use thereof in the manufacture of aluminium**
Tonerde-Reduktionszelle, Verfahren zur Herstellung einer solchen Zelle und ihre Anwendung bei der Herstellung von Aluminium
Cellule de réduction d'alumine, procédés de fabrication d'une telle cellule et son utilisation dans la production de l'aluminium

(30) Priority: 02.07.1979 GB 7922847
(43) Date of publication of application: 07.01.1981
(73) Proprietor: UNITED STATES BORAX & CHEMICAL CORPORATION, Los Angeles, California 90010 (US)
(72) Inventor: Biddulph, Richard Hampton, Surbiton Surrey (GB); Wickens, Anthony John, Surrey (GB); Creffield, Geoffrey Kenneth, Chessington Surrey (GB)
(74) Representative: Myerscough, Philip Boyd

## Description

This invention relates to an improved alumina reduction cell, to methods of producing such a cell, and to the use of the cell in the manufacture of aluminium.

Aluminium metal is prepared electrolytically by the reduction of alumina. Conventional alumina reduction cells comprise a vessel having a refractory lining, frequently of carbon, containing, as molten electrolyte, alumina dissolved in fused cryolite. The floor of the cell or vessel is typically made of a carbonaceous material, which not only provides thermal insulation, but also serves as part of the cathode. At least one anode is disposed within the vessel spaced apart from the cathode. Upon the passage of an electric current between anode and cathode, aluminium is formed by electrolytic reduction of the alumina. The molten aluminium formed is denser than the cryolite electrolyte and collects as a pool of metal on the floor of the cell. Molten aluminium metal is drained from the cell in order to prevent too deep a pool of aluminium metal forming on the floor of the cell. Quite clearly, the molten aluminium on the floor of the cell cannot be allowed to touch the anodes or short-circuiting of the cell would take place.

Molten aluminium does not readily wet carbonaceous materials. This can quite easily be demonstrated by allowing a drop of molten aluminium to contact an untreated surface of a carbonaceous substrate whereupon the aluminium will form a bead or globule and will not spread over the surface of the carbonaceous substrate. The fact that molten aluminium metal does not readily wet or spread over the floor of an alumina reduction cell can cause operating problems. The deeper is the layer of molten aluminium at the bottom of a cell, the greater necessarily must be the interelectrode distance. The greater is the inter-electrode distance the lower is the operating efficiency of the cell and the greater is the power requirement of the cell. Not only this, but the layer of molten aluminium formed upon an untreated carbonaceous cell floor is of sufficient thickness to permit thermal or magnetic currents to develop therein, making the layer somewhat unstable and liable to turbulence, so that waves can form in the layer and which can touch an anode and short-circuit the cell. The depth of the layer of molten aluminium at the bottom of a cell may vary from cell to cell, but typically is in the range from 3 to 8 centimetres.

Proposals have been made to modify the floor of an alumina reduction cell. For example, it is known that titanium and zirconium carbides are strongly wetted by molten aluminium and have good electrical conductivity and low solubility in molten aluminium. U.S. Patent Specification No. 3,471,380 (Bullough-issued 7th October 1969) describes a method of improving the performance of an alumina reduction cell by the formation of a coating of a beneficial metal carbide, in particular of titanium or zirconium, on the carbon cathode surface of the cell. The coating is produced by adding to electrolyte within the cell a refractory metal or compound thereof so that, during operation of the cell, a coating of a carbide of the metal forms upon the carbon cathode surface. However, refractory metal carbides do not provide ideal coatings for carbon substrates in an alumina reduction cell since they are susceptible to thermal shock.

U.S. Defensive Publication T993002 (Kaplan et a/-issued 1 st April 1980) discloses the provision of a titanium diboride surface to contact molten aluminium at the bottom of an alumina reduction cell. The titanium diboride surface is provided by refractory tiles secured to a carbonaceous substrate. The tiles are stated to be wettable by molten aluminium and to be chemically inert under the conditions of the electrolytic process. Although titanium diboride is less susceptible to thermal shock when titanium carbide and a titanium diboride surface would make possible considerable energy savings during operation of the alumina reduction cell, the tiles proposed for use in the Defensive Publication are of considerable thickness and therefore necessarily wasteful of titanium diboride, a very expensive material. Also problems arise from the need to bond the tiles to the carbonaceous substrate. The method of the Defensive Publication is considered to be so expensive in terms of the tiles required, that the ostensible cure would be worse than the complaint since greater expense would be incurred in fabricating and installing the tiles than could be saved by virtue of the reduced energy consumption of the alumina reduction process.

U.S. Patent Specifications Nos. 3,697,390 and 3,827,954 (McCawley et a/-issued 10th October 1972 and 6th August 1974, respectively) disclose the formation of platings of titanium, zirconium or hafnium borides on substrates by electrodeposition from fused borate baths. The anodes to be used comprise a metal of the desired boride or the boride itself. No mention is made in either Patent Specification of the deposition of metallic boride coatings on carbonaceous substrates, and the cathodes used in the Examples are all metallic, for example being of molybdenum, nickel or "Inconel". Japanese Laid-Open Patent Application 1974-67844 (Toyota-published 1 st July 1974) discloses a method of coating ferrous metals or their alloys with a titanium diboride layer by electrodeposition from a molten bath of a borate salt containing dissolved titanium. The reference states that the metal or alloy cathode to be used in the method must have a carbon content of less than 0.1 percent if a titanium carbide layer is not to be formed.

While therefore the prior art has recognised the desirability of providing an alumina reduction cell with a cathode, or cathode coating, that is readily wettable by molten aluminium and has suggested titanium diboride in this context, it has hitherto been considered that a layer of titanium diboride could not be formed on a carbonaceous substrated by electrodeposition without the formation of titanium carbide. We have now found surprisingly that a layer of titanium diboride can be formed upon a carbonaceous substrated by electrodeposition.

The invention accordingly provides an aluminium reduction cell comprising a vessel having a refractory lining and at least one anode disposed within said vessel, wherein at least part of the vessel floor severes as a cathode and said cathode comprises a carbon substrate having an adherent surface layer of electrodeposited titanium diboride.

The alumina reduction cell of the invention can be prepared by electrodepositing the titanium diboride layer on a carbonaceous cathode in situ in the cell, or by electrodepositing a layer of titanium diboride on at least one of the surfaces of carbonaceous blocks or elements externally of the cell and then installing the blocks or elements in a cell to provide the coated cathode surface. In the latter case the coated blocks or elements are positioned on the floor of cell and secured thereto with, for example, pitch.

An adherent surface layer of titanium diboride is formed in accordance with the invention, either on a carbonaceous cell floor or on constituent carbonaceous blocks or elements, by electrodeposition from a molten electrolyte consisting of a source of boron having titanium or a compound thereof dissolved therein. The carbonaceous cell floor or the blocks or elements serve as cathode and a firmly adherent surface layer forms thereon, with the electrodeposit of titanium diboride faithfully following the surface contours of the cathode. The anode preferably is of carbon since it has been found that better quality electrodeposits are formed with carbon anodes. It is, however, possible to use consumable titanium anodes which dissolve anodically to provide titanium values in the molten electrolyte. When using titanium anodes it is not necessary separately to dissolve a source of titanium in the molten electrolyte. If, however, a source of titanium is to be dissolved in the electrolyte, as for example when using carbon anodes, it is preferred to use titanium dioxide or a titanate as such a source. It is particularly preferred to use an electrolyte containing 2 to 10% by weight of titanium dioxide as a source of titanium. The molten electrolyte must contain a source of boron, and it is preferred to use an anhydrous borate as such a source, more particularly sodium tetraborate (borax) or potassium tetraborate. In general the molten electrolyte should be sufficiently conductive as to provide adherent electrodeposits of titanium diboride on the carbonaceous cathode and also sufficiently fluid as to permit ready removal from an electrolytic cell. When the electrodeposit of titanium diboride is formed in situ in an alumina reduction cell, the electrolyte should be removed and the cell cleaned.

The cell voltage should not exceed 2 volts if adherent electrodeposits are to be formed, but the conditions of the electrolysis for the deposition of the titanium diboride layer are otherwise not particularly critical. At voltages above 2 volts the electrodeposit becomes powdery and less adherent. Preferred voltages are from 1.2 to 1.8 volts. The current density can vary over a wide range and suitable values are from 5 to 100 milliamps per cm². The temperature should clearly be one at which the electrolyte is molten and of the requisite conductivity. Suitable temperatures are in the region of 900 to 1000°C. If necessary a flux can be added to the electrolyte to assist in operating at a desired temperature. The electrolyte desirably is agitated to assist in the formation of good quality deposits and agitation can conveniently be provided by means of a rotating anode. The duration of the electrolysis will be dependent to a large extent upon the thickness desired for the titanium diboride surface layer. Prolonging the electrolysis, replenishing the electrolyte as required, will result in the production of thicker electrodeposits. If desired, successive layers can be built up by repeated electrodepositions.

The titanium diboride layer can be electrodeposited directly onto an untreated carbonaceous cathode, but an underlayer of a titanium carbide electrodeposit can be provided if desired.

The surface layer of titanium diboride on the carbonaceous cathode of the alumina reduction cell of the invention not only is readily wetted by molten aluminium with the advantages referred to above, but also reduces the penetration of the cathode by sodium metal which can be formed during the alumina reduction. When sodium penetrates a carbonaceous cathode it can cause breakdown of the cathode.

The invention will now be illustrated by the reference to the following Examples.

### Example 1

An electrolyte consisting of 5% by weight TiO, and 95% by weight K₂8₄0₇ was electrolysed using graphite electrodes. The anode was also used as a stirrer. Electrolysis was continued for four hours at 950°C at 1.3 to 1.8 volts and a current density of 36 to 56 milliamps per cm² (m.a. cm⁻²).

After electrolysis the residual electrolyte was removed and the cathode was washed with water. X-ray diffraction showed the presence of titanium diboride and optical microscopy showed it to be present as a layer about 50 ,um thick. Wetting tests showed that it was readily wetted by molten aluminium.

### Example 2

An electrolyte containing 5% Ti0₂ by weight and 95% by weight Na₂B₄0, was electrolysed using a carbon cathode and a graphite anode for 3.5 hours at 950°C and at 1.3 volts and a current density of 60 to 100 m.a. cm-^{2.} After electrolysis the cathode was washed clean of electrolyte and examination by X-ray diffraction and optical microscopy showed the presence of an adherent titanium diboride layer.

### Example 3

Na₂B₄O₇ was electrolysed using a graphite cathode and a rotating titanium anode for 5 hours at 950°C at 1.5 volts and current density of 30 m.a. cm-². After electrolysis the cathode was washed clean of electrolyte and X-ray diffraction and optical microscopy showed the presence of an adherent titanium diboride layer.

### Example 4

An electrolyte containing 2% by weight Ti0₂ and 98% by weight K₂B₄O₇ was electrolysed using a graphite cathode and a titanium anode for five hours at 950°C at a voltage of 1.2 volts and a current density 5 m.a. cm-². After electrolysis the remaining electrolyte was removed and X-ray diffraction and optical microscopy showed the graphite cathode to be coated with a layer of titanium diboride with an estimated thickness 20 ,um.

### Example 5

K₂B₄O₇ was used as an electrolyte with a graphite cathode and titanium anode. This was electrolysed for 4.5 hours at 950°C at 1.5 volts and current density of 35 m.a. cm-². After electrolysis the remaining electrolyte was washed off. X-ray diffraction and optical microscopy showed the presence of a layer of titanium diboride on the surface of the graphite cathode with an estimated thickness 50 ,um.

## Claims

1. An alumina reduction cell comprising a vessel having a refractory lining and at least one anode disposed within said vessel, wherein at least part of the vessel floor serves as a cathode characterised in that said cathode comprises a carbon substrate having an adherent surface layer of electrodeposited titanium diboride.

2. A method of producing an alumina reduction cell as claimed in Claim 1, characterised in that a molten electrolyte consisting of a source of boron having titanium or a compound thereof dissolved therein is electrolysed at a voltage not exceeding 2 volts within an alumina reduction cell comprising a vessel having a refractory lining and at least one anode disposed within said vessel, at least part of the vessel floor bing formed of carbon and serving as a cathode, to form an adherent surface layer of titanium diboride on said cathode by electrodeposition.

3. A method of producing an alumina reduction cell as claimed in Claim 1 characterised by electrodepositing at a voltage not exceeding 2 volts an adherent surface layer of titanium diboride on at least one surface of a plurality of carbonaceous blocks from a molten electrolyte consisting of a source of boron having titanium or a compound thereof dissolved therein, and installing the resulting carbonaceous blocks in the vessel floor of an alumina reduction cell, said at least one surface of the blocks serving as the cathode surface of the cell.

4. A method according to Claim 2 or 3 characterised in that anhydrous borate is the source of boron.

5. A method according to Claim 4 characterised in that the borate is sodium or potassium tetraborate.

6. A method according to Claim 4 or 5 characterised in that the electrolyte has titania or a titanate dissolved therein and electrolysis is conducted using a carbon anode.

7. A method according to Claim 4 or 5 characterised in that the electrolysis is conducted using a consumable titanium anode which dissolves anodically in a melt initially consisting of an anhydrous borate.

8. A method according to any one of Claims 2 to 7 characterised in that electrolysis is conducted at 1.2 to 1.8 volts.

9. Use of an alumina reduction cell as claimed in Claim 1 or as produced by a method as claimed in any one of Claims 2 to 8 in the production of aluminium metal by the electrolysis of a molten electrolyte comprising alumina and cryolite.

## Patentansprüche

1. Tonerde-Reduktionszelle in Form einer Wanne mit feuerfester Auskleidung und zumindest einer in die Wanne reichenden Anode, wobei zumindest ein Teil des Wannenbodens als Kathode ausgebildet, ist, dadurch gekennzeichnet, daß die Kathode eine Kohle-Unterlage ist, auf der sich eine festhaftende Schicht von elektrolytisch abgeschiedenem Titandiborid befindet.

2. Verfahren zur Herstellung der Tonerde-Reduktionszelle nach Anspruch 1, dadurch gekennzeichnet, daß in einer Zellen-Wanne mit feuerfester Auskleidung und zumindest einer in die Wanne reichenden Anode, wobei zumindest ein Teil des Wannenbodens aus Kohle oder Kohlenstoff besteht und als Kathode geschaltet ist, eine geschmolzener Elektrolyt aus einer Quelle für Bor, der Titan oder eine Titanverbindung gelöst enthält, bei einer Spannung nicht über 2 V elektrolysiert wird, zur Bildung einer haftenden Schicht aus Titandiborid an der Kathode durch elektrolytische Abscheidung.

3. Verfahren zur Herstellung der Tonerde-Reduktionszelle nach Anspruch 1, dadurch gekennzeichnet, daß durch elektrolytische Abscheidung bei einer Spannung von nicht üver 2 V eine haftende Schicht von Titandiborid auf zumindest einer Fläche einer Vielzahl von Kohleblöcken aus einem geschmolzenen Elektrolyten, bestehend aus einer Quelle für Bor und darin gelöst Titan oder eine Titanverbindung, abgeschieden wird, worauf die so überzogenen Kohleblöcke in den Boden einer Tonerde-Reduktionszelle derart eingebaut werden, daß zumindest eine Fläche dieser Blöcke als Kathodenfläche der Zelle zu wirken vermag.

4. Verfahren nach Anspruch 2 oder 3, dadurch gekennzeichnet, daß als Quelle für Bor wasserfreies Borat angewandt wird.

5. Verfahren nach Anspruch 4, dadurch gekennzeichnet, daß das Borat Natrium- oder Kalium-tetraborat ist.

6. Verfahren nach Anspruch 4 oder 5, dadurch gekennzeichnet, daß im Elektrolyt Titandioxid oder ein Titanat gelöst ist und mit Hilfe einer Kohle-Anode elektrolysiert wird.

7. Verfahren nach Anspruch 4 oder 5, dadurch gekennzeichnet, daß mit einer Titan-Opferelektrode elektrolysiert wird, die sich anodisch in einer Schmelze auflöst, die anfänglich aus wasserfreiem Borat bestanden hat.

8. Verfahren nach Anspruch 2 bis 7, dadurch gekennzeichnet, daß die Elektrolyse mit einer Spannung von 1,2 bis 1,8 V durchgeführt wird.

9. Anwendung der Tonerde-Reduktionszelle nach Anspruch 1 oder hergestellt nach einem der Ansprüche 2 bis 8 bei der Aluminiumgewinnung durch Schmelzfluß-Elektrolyse von Aluminiumoxid und Kryolith.

## Revendications

1. Cellule de réduction d'alumine, comprenant un récipient possédant un revêtement réfractaire et au moins une anode disposée à l'intérieur dudit récipient, dans lequel au moins une partie du plancer du récipient sert de cathode, caractérisée par le fait que la cathode comprend un substrat de carbone possédant une couche superficielle adhérente de diborure de titane déposé par électrodéposition.

2. Procédé de fabrication d'une cellule de réduction d'alumine selon la revendication 1, caractérisé par le fait qu'un électrolyte fondu, consistant en une source de bore où est dissous du titane ou un composé du titane, est électrolysé à une tension ne dépassant pas 2 volts à l'intérieur d'une cellule de réduction d'alumine comprenant un récipient ayant un revêtement réfractaire et au moins une anode disposée à l'intérieur du récipient, au moins une partie du plancher du récipient étant formée de carbone et servant de cathode, pour former, par électrodéposition, une couche superficielle adhérente de diborure de titane sur la cathode.

3. Procédé de fabrication d'une cellule de réduction d'alumine selon la revendication 1, caractérisé par le fait qu'on dépose par électrodéposition, à une tension non-supérieure à 2 volts, une couche superficielle adhérente de diborure de titane sur au moins une surface d'un certain nombre de blocs charbonneux à partir d'un électrolyte fondu consistant en une source de bore où est dissous du titane ou un composé du titane, et qu'on installe les blocs charbonneux obtenus dans le plancer du récipient d'une cellule de réduction d'alumine, cette surface des blocs servant de surface de cathode pour la cellule.

4. Procédé selon l'une des revendications 2 ou 3, caractérisé par le fait que la source de bore est du borate anhydre.

5. Procédé selon la revendication 4, caractérisé par le fait que le borate est le tétraborate de sodium ou de potassium.

6. Procédé selon l'une des revendications 4 ou 5, caractérisé par le fait que l'électrolyte renferme en solution de l'oxyde de titane ou un titanate, et que l'électrolyse est conduite en utilisant une anode de carbone.

7. Procédé selon l'une des revendications 4 ou 5, caractérisé par le fait que l'électrolyse est conduite en utilisant une anode de titane consommable qui subit une dissolution anodique dans un bain consistant initialement en un borate anhydre.

8. Procédé selon l'une quelconque des revendications 2 à 7, caractérisé par le fait que l'électrolyse est conduite sous 1,2 à 1,8 volt.

9. Utilisation d'une cellule de réduction d'alumine selon la revendication 1, ou fabriquée par un procédé selon l'une quelconque des revendications 2 à 8, pour la production d'aluminium métal par électrolyse d'un électrolyte fondu comprenant de l'alumine et de la cryolite.
